

264  
29

2

## UNITED STATES PATENT OFFICE.

MATTHEW A. HUNTER, OF SCHENECTADY, NEW YORK, ASSIGNOR TO GENERAL ELECTRIC COMPANY, A CORPORATION OF NEW YORK.

## TUBULAR METALLIZED FILAMENT.

1,025,469.

Specification of Letters Patent.

Patented May 7, 1912.

No Drawing.

Application filed September 8, 1908. Serial No. 452,080.

*To all whom it may concern:*

Be it known that I, MATTHEW A. HUNTER, a subject of the King of Great Britain, residing at Schenectady, in the county of Schenectady, State of New York, have invented certain new and useful Improvements in Tubular Metallized Filaments, of which the following is a specification.

The object of my invention is to produce a new form of filament for incandescent lamps which is made up of modified carbon of that variety now well-known in the art as "metallized carbon," and it comprises this new form of filament and a novel process for making the same.

It will be recalled by those skilled in the art that in the manufacture of metallized carbon filaments as usually carried out (and as described in United States Patent 20 #916,905, granted March 30, 1909 to Willis R. Whitney), a "base filament" of carbon (usually obtained by carbonization of a squirted filament of cellulose out of contact with air) is given a carbonaceous coating by 25 a flashing or treating process consisting of heating the filament with current in hydrocarbon vapor and subjected to an extremely high temperature (such as may be obtained in a carbon tube electric furnace), believed 30 to be somewhere in the range of temperature between 2300 and 2700° C. This firing at a high temperature (the so-called "metallizing" process) brings about important changes in the characteristics of the 35 filament. As the improved properties of the metallized filament are chiefly due to the changes produced in the outer shell by the firing treatment, it will be seen that a filament consisting solely of this modified form 40 of carbon will possess advantages over the composite form of filament resulting from the procedure above set forth.

According to my invention, I produce a 45 filament consisting of a tubular shell of metallized carbon. Such a filament possesses all the properties of metallized carbon, and the absence of a core insures a filament possessed of a high resistance per unit of length. In making this tubular filament 50 I deposit the metallizable coating upon a core consisting of some substance which is refractory enough to bear heating to the temperatures necessary in the treating proc-

ess but volatilizable at the high temperatures obtainable in a carbon tube furnace. 55 If suitable core material is used, the high heat treatment, or metallizing completely eliminates the core, leaving the metallized shell intact. I have found that titanium carbid is suitable for use in this manner as a 60 core material. I do not wish, however, to be limited to the use of this particular material, as other substances, as for example, zirconium carbid and other carbids, or even platinum, may also be used. 65

Although my invention is of general application, I will explain my process with particular reference to the production of a tubular filament using titanium carbid for the core material.

The novel features of my invention are pointed out with particularity in the claims appended to this specification.

For the production of a filament of titanium carbid I make use of the fact that 75 titanium dioxid, when heated in the presence of carbon, undergoes reduction with the formation of titanium carbid and carbon monoxid. The procedure is as follows: pure titanium oxid,  $TiO_2$ , is finely powdered and 80 mixed with some form of carbon, as graphitized lampblack, together with a carbonizable binder, such as glucose. The plastic mixture thus obtained is then squirted into filament-shaped threads. These threads are 85 baked in an oven heated to about 300° C., whereby the glucose is carbonized and the threads made conductive. The threads are then heated, as by means of a current passed, through them, with the result that the carbon serves to reduce the oxid with the formation of titanium carbid and liberation of 90 carbon monoxid. If the plastic mixture has been so compounded as to include theoretical quantities of carbon and  $TiO_2$ , the chemical 95 reaction will take place as follows:



The titanium carbid filaments so obtained are coherent and refractory. These filaments are next placed in an atmosphere of hydrocarbon vapor, such as benzine, and heated for about five seconds at a temperature of 1500 to 2000° C., which is above bright red heat. This heating may be accomplished by passing a current directly

through the filament in the usual way and produces a deposition of carbon on the titanium carbid core. This coating can be built up to any desired thickness. These 5 filaments with a coating of deposited carbon forming an outer shell are then packed with flaked graphite in suitable boats, or containers, and placed in a metallizing furnace. They are there heated for about twenty 10 minutes at the highest temperature obtainable in a carbon tube furnace, which I should estimate would be about 3500°. Upon removal of the filament from the metallizing furnace it is found that the titanium carbid core has vaporized, leaving the outer shell intact. This shell is shiny gray 15 in color and very dense and uniform. In fact, it seems to be and undoubtedly is of the same nature as the shell of an ordinary 20 commercial "metallized" filament. Such hollow filaments being uniform throughout have the advantage of freedom from thermal strains. They are operative at high efficiency and are otherwise well adapted for 25 general use in incandescent lamps.

What I claim as new and desire to secure by Letters Patent of the United States, is—

1. The method of producing a tubular conductor of metallized carbon, which consists in first producing a composite conductor consisting of a vaporizable core and a metallizable carbonaceous shell, and then firing said conductor at a temperature sufficient to vaporize said core and metallize said shell. 35

2. The method of producing a tubular conductor of metallized carbon, which consists in first producing a composite conductor consisting of a core of titanium carbid and a shell of carbonaceous material, and firing said conductor at a temperature sufficient to metallize the shell of carbonaceous material and vaporize out the core of titanium carbid. 40

In witness whereof, I have hereunto set 45 my hand this 5th day of September, 1908.

MATTHEW A. HUNTER.

Witnesses:

BENJAMIN B. HULL,  
MARGARET A. DELEHANTY.

---

Copies of this patent may be obtained for five cents each, by addressing the "Commissioner of Patents, Washington, D. C."

---